

# UNITED STATES PATENT OFFICE.

CARLETON ELLIS, OF MONTCLAIR, NEW JERSEY, ASSIGNOR TO ELLIS-FOSTER COMPANY, A CORPORATION OF NEW JERSEY.

## PROCESS OF MAKING BRIQUETS OR OTHER MOLDED ARTICLES.

1,246,805.

Specification of Letters Patent. Patented Nov. 13, 1917.

No Drawing.

Application filed March 28, 1913. Serial No. 757,301.

To all whom it may concern:

Be it known that I, CARLETON ELLIS, a citizen of the United States, and a resident of Montclair, in the county of Essex and State of New Jersey, have invented certain new and useful Improvements in Processes of Making Briquets or other Molded Articles, of which the following is a specification.

10 This invention relates to a method of making briquets and other solid or plastic bodies by means of sulfite waste liquor as a binding material and to the product of such method, all as more fully hereinafter set forth.

15 Sulfite waste liquor in a concentrated or solid form has been proposed as a binding material for briquets and the like, but being soluble in water briquets made from it will not stand the action of wet weather as when exposed to rain in open cars during transportation. Pitch and tar have been suggested as waterproofing agents for the sulfite liquor but owing to the smoke and soot produced by these there is little likelihood of general acceptance of binders of this character.

20 Many attempts have been made to render sulfite liquor waterproof but so far as I know, no satisfactory method to this end for making briquets and plastics has been devised.

25 I have found that the concentrated liquor especially the more acid types of the sulfite waste liquor are capable of being precipitated by lime to form a perfectly insoluble body, so far as this art is concerned, and which enable briquets to be prepared which resist the disintegrating effects of water to the degree desired. It is of course somewhat remarkable that sulfite waste liquor consisting so largely of lime compounds should be precipitated by quicklime or hydrated lime, but such is the case, especially 30 with the slightly acid varieties of the liquor. The liquors obtained from raw materials containing a rather high percentage of magnesia are preferable.

35 The product may be used for making flooring compounds, artificial stone, columns, and all sorts of plastics, as will now be evident.

In carrying out the method I take sulfite

liquor preferably of an acid character, such as may be made by concentrating in an acid condition or partially neutralized state, or by acidifying the neutral concentrate. I do not mean to exclude the neutral or alkaline, or hydrolyzed, or other forms or derivatives of sulfite waste liquor or spruce or other cellulosic liquors of a substantially equivalent character from the viewpoint of the present invention. The liquor is mixed with the materials to be bound together as coal dust or fines, culm, sawdust, mineral fillers, talc, magnesite, crushed rock, sand, fiber, asbestos, and the like, and then the lime in a finely divided condition is admixed therewith. Reaction takes place almost immediately with some liquors and the insoluble compound is formed in and around the filling material. Sometimes the reaction is not immediate especially when the sulfite liquor is diluted with 20 to 50% of water or when the sulfite liquor solids are because of the nature of the concentration in a less unstable condition. Thus in various ways the setting time may be controlled so that opportunity is afforded to work the plastic into suitable shape after mixing. Hydrated lime works usually a little slower than quicklime. About 50% of lime reckoned on the weight of sulfite liquor of 30 degrees Baumé is a satisfactory amount of precipitant. 30% and even less will serve but the setting time is greatly protracted, which of course for some purposes may not be undesirable. From 30-50% is however recommended for general operation. This may be exceeded in some cases.

40 In preparing a briquet from culm or coal material of various sorts the sulfite liquor may be mixed with this material to uniformly coat the particles thereof and the lime in fine powder may then be admixed, or the coal may first be floured with the lime and the sulfite liquor then added and thoroughly incorporated, briquetting following as soon as possible. Or the lime may be added in the form of the hydrate dry or as a paste or as milk or cream of lime. To secure the best results briquetting or forming into shape should take place before material setting has occurred.

45 The action of the lime or other precipitant employed is that of true precipitation or

coagulation, as the product in its preferred form is unattacked by boiling water although the sulfite liquor in the acid form preferably used is readily soluble in cold water.

On the weight of the coal employed from 6 to 10 per cent. of sulfite liquor may be used, the proportion varying between these or other limits according to the character of the coal amount of briquetting pressure and so forth. The coal particles need not be uniformly coated with the sulfite liquor provided sufficient of the latter be present to secure the required bonding effect.

15 Tests made with such briquets by exposing to a strong spray of water showed a plain sulfite liquor briquet to fall to pieces in 10 minutes while the limed product resisted perfectly for a period of four hours when the test was discontinued.

Although the reaction takes place readily in the cold with the lime reagent as above, heat may be employed if desired to modify the reaction. When precipitants other than 25 lime are used the conditions should be adjusted to meet any modification of the reaction under the circumstances. Similarly although the process is described more particularly with reference to the production of briquets it will now be evident that the reaction may be applied to other fields where it is desired to precipitate sulfite liquor to yield an insoluble product, especially as distinguished from "salting out" procedures

35 known in the art. Thus flooring, tool handles, blocks, and all kinds of molded products may be obtained. Added to paper stock in the beater engine, the sulfite liquor may be thrown down with lime or similar precipitant, giving a sizing material which serves for some of the darker shades of paper at least, and such size may be used in conjunction with rosin or other size if desired.

45 For convenient shipment and for certain other reasons including readiness with which the material may be incorporated with the coal or similar stock, the sulfite liquor may be dried to a solid and ground to a powder or dried in an atomizing system which yields the material in a pulverulent condition. This powder is then mixed with the coal, lime being added either before or after or with such mixture, and water incorporated 55 so as to cause the reaction either in the bulk mass or after forming into briquets.

Similarly a pulverulent product consisting of a mixture of the dry sulfite liquor solids and hydrated lime may be prepared 60 for use as a binder.

Other precipitants than lime may be employed as stated. Preferably however a basic body such as lime or barium hydrate is recommended and preferably with the 65 acid sulfite of cellulose waste liquor, it being

desirable to have only a moderate degree of acidity to permit of the reaction taking place with effectiveness.

Barium hydrate is not so powerful a precipitant as calcium hydrate, on some liquors. 70 Lime is a specific precipitant.

Another consideration is that in the case of briquets it becomes necessary to consider the ash of the fuel. Any addition of sulfur compounds such as pyrite is of course regarded as objectionable, while lime is even advantageous as it softens the clinker rendering same less likely to freeze to the stove fire box or grates. With 6% of sulfite liquor and 3% of lime the resulting ash is not objectionable in the case of most grades of coal, 80 both anthracite and bituminous.

Finally in recapitulation it should be stated that although I lay claim broadly to the novel reaction hereinbefore set forth, I 85 principally indicate concentrated acid sulfite liquor diluted as may be desired, as a binding material, precipitated by means of the specific precipitant quicklime or lime material, as calcium saccharate and the like, such 90 acid sulfite liquor being preferably in a colloidal and unstable form due to such concentration under these conditions so that the act of neutralization or over neutralization (an excess of precipitating agent being 95 preferably employed) induces not merely chemical combination but a polymerization or some similar form of coagulation the exact nature of which I do not herein attempt to describe. While lime exerts this effect 100 calcium chlorid does not yield the same results. Probably the removal of the excess of sulfite liquor and possibly some in combination with the solids of the liquor, which occurs during the treatment connected with 105 concentration, places the solids or some of them in an unstable condition and the addition of the lime by further combination under these peculiar conditions causes the effects observed. The bulking agent or material hereinafter mentioned is the material employed as the filler or the essential material to be bound together as aforesaid.

It will be readily understood that, by the concentration of waste sulfite liquor, the 110 product is rendered substantially free from sulfurous acid so that the action of sulfurous acid on the added lime is avoided, and sulfur, which is objectionable in briquets, is reduced to a minimum. It will also 115 be readily understood from the foregoing description that, by reason of the chemical reactions which take place during concentration, the constituents of the sulfite liquor which are acted upon by the lime in my 120 process, are in a chemically unstable condition as compared with their condition in unconcentrated sulfite liquor so that, upon the addition of lime, the negative ions of the precipitant are seized upon with peculiar 125

avidity and a different product obtained from that resulting from the action of lime upon unconcentrated sulfite liquor.

I do not herein claim the following subject matter disclosed herein, which matter is claimed in the copending applications noted below:—

The dried acid solid dried sulfite waste liquor, and the general process of making such material, claimed in application 779,516, filed July 17, 1913.

The use of such material as a tanning agent, claimed in application 162,941 filed April 18, 1917.

15. Briquets and formed articles generally, made with acid solids of sulfite waste liquor dried by atomization, claimed in application 165,441, filed April 30, 1917.

The dried comminuted waste sulfite liquor solids, claimed in application 167,332, filed May 8, 1917.

The acid solution made by redissolving the dried solids, claimed in application 168,275, filed May 12, 1917 and application 25. 186,481 filed August 16, 1917.

The use of the somewhat acid solids, dried by atomization in making briquets and other formed articles, claimed in application 176,280 filed June 27, 1917.

30. In mixing the materials of which briquets and similar objects are formed, particularly if mixed in a dried state with the addition of water, it may frequently happen that some portion of the liquor solids do not react with the lime to produce an insoluble product. Since, however, a material part, at least of such solids would be rendered insoluble, I use in one of the appended claims, the expression "insolubilizing at least a portion of the solids of the binder."

In order to clearly differentiate between such very slow and gradual insolubilizing of the liquor solids, which to a certain extent may occur under service conditions per-

haps by atmospheric oxidation thereof, and my invention in which the insolubilization of the liquor solids is effected within a relatively short time, as by the addition of lime or equivalent material at the time of forming the product, I use the expression "artificially insolubilizing said liquor solids."

What I claim is:—

1. The process of making briquets or other molded articles which comprises mixing concentrated acid sulfite cellulose waste liquor with a bulking material containing coal dust and fragments and incorporating quicklime material.

5. The process of making briquets or other molded articles which comprises mixing concentrated acid sulfite cellulose waste liquor or its solids with a bulking material and a precipitant for the liquor solids.

3. The process of making briquets or other molded articles which comprises mixing concentrated acid unstable sulfite cellulose waste liquor with a bulking material and quicklime material.

4. The process of making briquets or other shaped articles which comprises incorporating concentrated sulfite cellulose waste liquor or its solids with a bulking material and in artificially insolubilizing said liquor solids.

5. A process of making a shaped article 75 from a bulking material and an acid binder containing the solids of concentrated sulfite cellulose waste liquor, which comprises incorporating said two materials together and insolubilizing at least a portion of the solids 80 of the said binder.

Signed at Montclair, in the county of Essex and State of New Jersey, this 24th day of March, A. D. 1918.

CARLETON ELLIS.

Witnesses:

A. A. WELLS,  
N. L. FOSTER.